

## UNITED STATES PATENT OFFICE

2,159,973

## GELATINIZED HIGH EXPLOSIVE COMPOSITION AND METHOD OF PREPARATION

Walter Eastby Lawson, Woodbury, N. J., assignor to E. I. du Pont de Nemours &amp; Company, Wilmington, Del., a corporation of Delaware

No Drawing. Application April 1, 1938,  
Serial No. 199,446

13 Claims. (Cl. 52—13)

This invention relates to the preparation of gelatinized high explosives, and more particularly to the acceleration of the gelatinization of nitrocellulose with nitroglycerin and with nitroglycerin solutions of aliphatic nitric esters or 5 nitrocompounds.

It is known that, when certain otherwise desirable nitrated materials are present dissolved in the nitroglycerin, the gelatinization of the 10 solution with nitrocotton is undesirably slow and in many cases incomplete. When such incomplete gelatinization takes place, the finished explosive is unsatisfactory in its properties and deteriorates markedly under conditions of long 15 time storage, particularly from the point of view of consistency and plasticity of the gelatinized material and exudation of nitroglycerin therefrom. This problem has been studied previously, and proposals have been made for its solution, 20 for example by Moran in U. S. Patent 1,640,712 and by Fassnacht in U. S. Patent 1,966,090.

The object of the present invention is a new and improved high explosive composition containing a gelatinized liquid nitric ester of superior properties. A further object is such a composition in which the gelatinization with nitrocellulose has been accelerated and the properties of the finished product thereby improved. A still further object is a novel process for bringing about the aforesaid accelerated gelatinization. Additional objects will be disclosed as the invention is described more at length herein-after.

I have found that the foregoing objects are 35 accomplished by incorporating with the nitroglycerin an acid amide of a monobasic fatty acid or an alkyl derivative thereof. The acid amide for use according to my invention will have the formula



40 in which  $R_1$ ,  $R_2$ , and  $R_3$  consist either of hydrogen or an alkyl radical. As an example, 45 formamide and its alkyl derivatives are very desirable accelerants according to my invention, in which case  $R_1$  represents hydrogen. When  $R_1$  represents a  $CH_3$  group, the accelerant will be 50 acetamide or an alkyl derivative thereof.  $R_2$  and  $R_3$ , likewise, may represent either hydrogen or alkyl groups. As specific examples of compounds 55 advantageous for use as gelatinization accelerants, I may cite formamide ( $H-CO-NH_2$ ), acet-

amide ( $CH_3-CO-NH_2$ ), monomethylformamide

5

dimethylformamide



10

dimethylacetamide ( $CH_3-CO-N-(CH_3)_2$ ), diacetamide ( $(CH_3-CO)_2-NH$ ), propionamide, butyramide, and many others.

It is important to note that dimethylformamide 15 is the preferred gelatinization accelerant according to the present invention. It should be understood that this particular compound is not merely the equivalent of the others listed but is superior thereto.

The use of a gelatinization accelerant of the 20 acid amide type, according to my invention, will have advantages in gelatinized nitroglycerin high explosives generally but will be particularly efficacious where tetranitrodiglycerin is present in solution in nitroglycerin, since such solutions 25 attain outstanding improvement thereby. The invention is applicable with high efficiency in the case of the standard straight and ammonia gelatin dynamites, as well as with the so-called semi-gelatins, where smaller percentages of nitrocellulose are present and less complete gelatinization 30 is effected. By its utilization, not only does acceleration result, but a more uniform and completely gelatinized product is obtained.

For a more exact understanding of my invention, the process of producing the improved gelatinous high explosives is illustrated below.

## Example 1

The amounts of ingredients used in this example are based on the production of a 100 lb. 40 mixing of an ammonia gelatin dynamite. 25 lbs. of nitroglycerin, containing dissolved tetranitrodiglycerin, was introduced into the bowl in which the mixing was made, and 0.25 lb. dimethylformamide was added to the nitroglycerin and dissolved therein. 0.65 lb. of a suitable nitrocotton was then introduced into the nitroglycerin. The mixture was agitated, while maintaining the 45 temperature at approximately 120° F. When the solution had thickened or gelatinized to the proper degree, the solid ingredients of the dynamite, already thoroughly mixed, were added for incorporation. These ingredients comprised 50 approximately 7.8 lbs. ammonium nitrate, 51.2 lbs. ammonium nitrate, 55

lbs. sodium nitrate, 14.6 lbs. combustible dope ingredients, and 0.5 lb. chalk. After the addition of these latter ingredients, the mixing was continued until the finished explosive was of the proper consistency. It was then removed from the bowl and cartridge in the usual manner.

*Example 2*

- 10 For the manufacture of a 100 lb. mixing of a semi-gelatin containing a gelatinization accelerant according to my invention, 20 lbs. of nitroglycerin was introduced into the mixing bowl, and 0.15 lb. of dimethylformamide and 0.20 lb. nitrocotton were introduced into, and incorporated with, the nitroglycerin, as in Example 1. The proper amounts of solid ingredients were then thoroughly mixed with the liquid ingredients, a temperature of approximately 120° F. again being maintained.
- 15 The explosive compositions made in accordance with my invention possessed very marked superiority, not only over similar compositions containing no specific gelatinization accelerant, but also over compositions containing accelerants of the prior art. In the case of 40% ammonia gelatins, for example, containing the accelerant of my invention and tetra-nitrodiglycerin dissolved in the nitroglycerin, the explosive was free from leakiness after long-time storage under severe conditions and retained its initial high degree of plasticity. Similar retention of the initial desired properties was observed in the case of the semi-gelatins, also, and other gelatinous high explosives.
- 20 The increased acceleration of gelatinization brought about by operation according to my invention may be strikingly illustrated by the results of some small-scale gelatinization tests, where the time of flow of gelatinized nitroglycerin was measured when different accelerants were used. Using 50 grams of nitroglycerin and sufficient nitrocotton to give the desired range of flow speeds, the weights of material required for the same rate of flow, and consequently for the same
- 25 degree of acceleration, were as follows:—

|                                | Grams |
|--------------------------------|-------|
| Dimethylformamide              | 0.15  |
| Ethylene glycolmonoethyl ether | 0.40  |
| Dinitrotoluene                 | 4.50  |

50 The superiority of dimethylformamide as an example of my invention is illustrated in the above, since only 0.15 gram produced an acceleration equivalent to 0.40 gram of one of the best accelerants of the prior art. This improvement will be appreciated when it is realized that, with no accelerant present, the amount of nitrocotton used in the foregoing experiments was insufficient to produce the same stage of gelatinization in 24 hours, whereas the results cited were obtained over an interval of 20 minutes.

55 Varying amounts of the acid amide accelerant may be used, preferably in an amount between 0.1 and 5.0% of the nitroglycerin present. My preferred range is between 0.5 and 2.0% of the weight of nitroglycerin.

60 In carrying out my invention and obtaining the consequent improved properties, nitroglycerin may be used alone as the liquid explosive nitric ester, if desired. Likewise, other liquid nitric esters may be employed, such as ethylene glycol dinitrate, either by itself or with nitroglycerin. Furthermore, various other nitric esters and nitrocompounds may be present also, dissolved in 65 the liquid nitric ester, thereby imparting vary-

ing properties to the liquid explosive, such as improved resistance to freezing, etc. Such added nitrated materials may be cited as tetranitrodiglycerin, nitrated sugars, nitrochlorhydrins, aromatic nitrocompounds, and the like. While I have described the use of an acid amide according to my invention as the sole accelerant, it should be understood that I may, if desired, also employ such an amide together with an accelerant of the prior art, for example ethyleneglycol monoethyllether, and thereby gain important advantages.

65 It will be understood that many variations, in details and in compositions, from those described in the foregoing may be made without departure from the scope of my invention. I intend to be limited, therefore, only by the following patent claims.

I claim:

1. A high explosive composition comprising a liquid explosive nitric ester gelatinized by means of nitrocellulose, and an acid amide having the formula



25

in which R<sub>1</sub>, R<sub>2</sub>, and R<sub>3</sub> are taken from a group consisting of hydrogen and the alkyl radicals.

2. A high explosive composition comprising a liquid explosive nitric ester gelatinized by means of nitrocellulose, and a gelatinization accelerant taken from the group consisting of the acid amides of the monobasic fatty acids and their alkyl derivatives.

35

3. The explosive composition of claim 2, in which the gelatinization accelerant is formamide.

4. The explosive composition of claim 2, in which the gelatinization accelerant is acetamide.

5. The explosive composition of claim 2, in which the gelatinization accelerant is dimethylformamide.

40

6. A high explosive composition comprising a solution of tetranitrodiglycerin in nitroglycerin, said solution being gelatinized by means of nitrocellulose, and a gelatinization accelerant taken from the group consisting of the acid amides of the monobasic fatty acids and their alkyl derivatives.

45

7. A gelatinized nitroglycerin high explosive comprising nitroglycerin and nitrocellulose, and a gelatinization accelerant taken from the group consisting of the acid amides of the monobasic fatty acids and their alkyl derivatives, said accelerant being present in an amount between 0.1 and 5.0% of the nitroglycerin present.

55

8. The process of accelerating the gelatinization of nitrocellulose with a liquid explosive nitric ester, which process comprises bringing about said gelatinization in the presence of an acid amide having the formula



65

in which R<sub>1</sub>, R<sub>2</sub>, and R<sub>3</sub> are taken from the group consisting of hydrogen and the alkyl radicals.

9. The process of accelerating the gelatinization of nitrocellulose with nitroglycerin containing dissolved tetranitrodiglycerin, which process comprises bringing about said gelatinization in the presence of a gelatinization accelerant taken from the group consisting of the acid amides of the monobasic fatty acids and their alkyl derivatives.

75

10. The process of accelerating the gelatinization of nitrocellulose with a liquid explosive nitric ester, which process comprises bringing about said gelatinization in the presence of dimethylformamide.

11. The process of accelerating the gelatinization of nitrocellulose with nitroglycerin, which process comprises bringing about said gelatinization in the presence of dimethylformamide in an amount between 0.1 and 5.0% of the nitroglycerin present.

12. A high explosive composition comprising ethylene glycol dinitrate gelatinized by means of nitrocellulose, and a gelatinization accelerant taken from the group consisting of the acid amides of the monobasic fatty acids and their alkyl derivatives. 5

13. The explosive composition of claim 12 in which the gelatinization accelerant is dimethylformamide.

WALTER EASTBY LAWSON. 10